

## UNITED STATES PATENT OFFICE

ROBERT J. ANDERSON, OF FAIRMONT, WEST VIRGINIA, ASSIGNOR TO FAIRMONT MANUFACTURING COMPANY, OF FAIRMONT, WEST VIRGINIA, A CORPORATION OF WEST VIRGINIA

## PROCESS OF TREATING METALS WITH NITROGEN

No Drawing.

Application filed May 1, 1928. Serial No. 274,361.

My invention relates particularly to a process of treating molten metals, including alloys, etc., with nitrogen, and has relation especially to the treatment of the metals, particularly aluminum and its alloys, in this way to improve their physical characteristics.

Molten metals, by which I mean to include alloys, and especially aluminum and its alloys, may, and usually do, contain dissolved gases and other impurities, such as foreign suspended matter. The dissolved gases present therein depend upon the conditions under which the same is melted, the process of manufacture, etc., and, generally speaking, the gases present cannot be controlled effectively, or at all, under the conditions of manufacture. Where dissolved gases are present the effect is to cause porosity in the castings made therefrom, which is, of course, of great moment in foundry practice as it leads to rejection of castings, porosity, weakness, breakages, etc. It is found that metals dissolve increasing quantities of gases with increasing temperature of melting, thus departing from Henry's law which applies to other liquids. Also, such metal-gas solutions tend to remain saturated. That is to say, as the temperature is decreased from a high temperature the molten metal does not give off gas at the same rate at which the gas was taken up, and, on solidifying, there is a tendency for a considerable volume of gas to be evolved, causing blow-holes and porosity.

I have discovered that these gases, and, also, other deleterious suspended solid impurities, by which term I mean to include solids which become molten or not when the body of metal is melted, may be removed by treatment of the metal with nitrogen, which is only dissolved with difficulty by the metal at a given temperature and which does not combine to an undesirable extent with the metal itself.

The object of my invention is, therefore, to remove such gases and other deleterious matters from metals in the above manner. The theory of the action of the removal thereof is not entirely known but it is believed that the action comprises mainly the

removal of the dissolved gases and other deleterious impurities mechanically by agitation due to the introduction of the nitrogen gas, as above referred to, although there may be, also, some combination brought about with the dissolved gases, or other deleterious impurities, as well. The deleterious solid impurities which are removed in this way are of various kinds, according to the particular kind of metal treated. These comprise, for example, sonims in steel, oxides in brass and bronze, dirt, nitride, carbide and oxide in aluminum, all of which have a deleterious effect on the mechanical characteristics of the metals. For instance, in the case of steel, it has been found that dirty steel, containing some slag enclosures, is much inferior in its properties to the steel from which these solid impurities have been removed. In fact, such inclusions have a harmful effect on the fatigue range, impact resistance and other mechanical properties of the steel. Also, in the case of aluminum and its alloys, particularly its light alloys, I have demonstrated that clean aluminum, made by being subjected to my process, has very superior mechanical properties as compared with aluminum which has not been subjected to treatment in my process. The same is true in regard to the other metals. In fact in all such metals, not only do solid non-metallic impurities produce zones of weakness around the inclusions, as referred to, but such impurities, when present even in relatively small percentages, have been found to have a profound influence on the mechanical properties, as well as on the working, rolling and casting qualities of the metals. Also, the metal so treated is found to have greatly increased strength and to be capable of much greater elongation. In fact, it has been found previously substantially impossible to remove or reduce by any previously known method, small percentages of impurities such as can be removed by my process. I have found that even very small percentages of impurities may be practically entirely removed by treatment in my process.

While my invention is capable of embodiment in many different forms, for the pur-

pose of illustration I shall describe only certain forms of my invention hereinafter.

For example, in carrying out my invention I find nitrogen to be very useful in the treatment of metals generally, such as those listed above, but it is especially applicable to the treatment of aluminum and its light alloys. For instance, in treating aluminum I provide a bath of molten aluminum which may have any desired temperature, such, for example, as 700° C. or above, and then apply the nitrogen gas to the metal as by bubbling it through the molten metal, thus causing agitation of the molten metal, until the impurities are substantially entirely removed. This causes flotation of the solid impurities due to the surface tension of the metal which sustains the impurities on the top of the body of metal. Thus, the introduction of say 1 cu. ft. of nitrogen, referred to standard conditions of temperature and pressure, per 300 lbs. of metal, may be ample to remove dissolved gases and foreign suspended matter, after which the metal may be poured to form a finished or semi-finished casting. In this treatment the gas may be applied to the metal in any desired way and in any desired type of apparatus, but, for example, the gas may be injected into the metal with the aid of a perforated pipe, which may be located in the metal in such a way that the perforations therein for the discharge of the nitrogen are located at the bottom of the body of molten aluminum. The nitrogen does not combine with the aluminum appreciably at the working temperature referred to but removes the dissolved gases and other deleterious impurities, some of which may have combined with the nitrogen to some extent, but which are in any case effectively removed by the treatment. The dissolved gases pass off into the atmosphere while the solid inclusions join the top slag or dross and may be removed by skimming. In the case of aluminum the impurities present may be reduced in this way to practically nil.

While I have described my invention above in detail I wish it to be understood that many changes may be made therein without departing from the spirit of the same.

I claim:

1. The process which comprises removing a solid impurity from a metal by the intermingling of nitrogen therewith until the solid impurities are substantially entirely removed.

2. The process which comprises removing a solid impurity from aluminum by the intermingling of nitrogen therewith until the solid impurities are substantially entirely removed.

3. The process which comprises removing a solid impurity from a metal by the intermingling of nitrogen therewith, thereby agitating the metal to free the impurities there-

from until the solid impurities are substantially entirely removed.

4. The process which comprises removing a solid impurity from a metal by the intermingling of nitrogen therewith and the flotation of the impurity due to the surface tension of the metal until the solid impurities are substantially entirely removed.

5. The process which comprises removing a solid impurity from aluminum by the intermingling of nitrogen therewith and the flotation of the impurity due to the surface tension of the metal until the solid impurities are substantially entirely removed.

6. The process which comprises removing a solid impurity from a metal by the intermingling and combining of nitrogen therewith until the solid impurities are substantially entirely removed.

In testimony that I claim the foregoing, I have hereunto set my hand this 28th day of April, 1928.

ROBERT J. ANDERSON.

90

95

100

105

110

115

120

125

130